

June 4, 1935.

E. HEDIGER

2,003,592

GLAZE FOR NONMETALLIC RESISTORS

Filed Jan. 3, 1933



INVENTOR.  
ERNST HEDIGER  
BY *Al Benner*  
ATTORNEY

## UNITED STATES PATENT OFFICE

2,003,592

## GLAZE FOR NONMETALLIC RESISTORS

Ernst Hediger, Niagara Falls, N. Y., assignor to  
 Globar Corporation, Niagara Falls, N. Y., a corporation of New York

Application January 3, 1933, Serial No. 649,968

4 Claims. (Cl. 201—76)

This invention relates to coatings for resistors which are subjected to oxidizing conditions during their operation, and particularly to methods of improving the electrical properties and useful life of resistors composed principally of silicon carbide. The invention has for one of its objects the solving of certain problems encountered in the operation of rigid self-sustaining heating elements at high temperatures, and is particularly applicable to resistors composed of relatively coarse particles. Coatings made in accordance with my invention materially increase the strength of the resistor and also minimize the change in electrical resistance and change in resistance temperature characteristics which often take place in the operation of high temperature heating elements.

The changes, apart from direct mechanical breakage, which limit the useful life of resistors composed of silicon carbide or other carbides are not in general obvious upon visual examination of the cold resistor. There is, however, a distinct change after a period of use which is usually manifested by an increase in resistance or by a change in the temperature resistance characteristic of the resistor. The changes in electrical properties take place even at relatively low temperatures where there is no apparent oxidation of the resistor material.

An increase in resistance of the resistor rod permits less current to flow through the rod at a given voltage, so that the resistor, after a certain period of use, fails to heat up to the temperature which is originally attained and which is desired. This effect finally becomes so pronounced that the resistor must be replaced. One of the effects of my type of coating is to retard this change.

Another typical change accompanying the aging of a resistor is the development of a negative resistance temperature coefficient. This means that the resistance becomes less as the temperature increases. The existence of this negative relationship has long retarded the application of this type of resistor to many heating problems because unless the voltage is reduced as the rod becomes hot there is a tendency for the resistor to "run away" and destroy itself through overheating. As described in my copending application, Serial No. 575,665, filed Nov. 17, 1931, Patent 1,906,853, May 2, 1933, I have found it possible to produce a resistor having a positive temperature coefficient of resistance by certain specific burning methods and by the use of certain types of silicon carbide. Such resistors are substantially devoid of materials other than silicon carbide, and are bonded by a process known in the art as self-bonding or "recrystallization". Even with these resistors, however, the resistance temperature coefficient becomes less positive and may even become negative after a long period of service. I have found that the use of my coating materially delays the alteration of this characteristic.

My invention is illustrated by the accompanying drawing which shows a section taken in a plane perpendicular to the longitudinal axis of one of my improved resistors.

As indicated in the drawing, the body of the resistor contains comparatively coarse granules 3, and is surrounded by a coating 2 which is relatively much more compact and which is described in detail below.

The following table illustrates the manner in which a coating of the type composing my invention improves the properties of recrystallized silicon carbide resistor rods designed for use on 110 volt circuits with a current of 10 amperes. The resistors in question are 14 inches long and  $\frac{3}{8}$  of an inch in diameter.

| Test No. | Character of element | Transverse strength lbs./sq. in. | Increase in resistance after 1,000 hours |    |
|----------|----------------------|----------------------------------|------------------------------------------|----|
|          |                      |                                  | Per cent                                 | 30 |
| I.....   | Uncoated.....        | 2000                             | 22                                       |    |
|          | Coated.....          | 4000                             | 14                                       |    |
| II.....  | Uncoated.....        | 2500                             | 26                                       |    |
|          | Coated.....          | 4200                             | 12                                       |    |

These results show a notable increase of strength in the coated resistors as compared with the uncoated resistors. The results show also that the coated resistors retain their electrical characteristics better than uncoated resistors up to 1,000 hours of use.

The increase in mechanical strength secured through the addition of a surface coat to the resistor is particularly advantageous because it permits the use of materially coarser granules in the body of the resistor, a practice that results in a reduction of the rate of oxidation of the resistor at elevated temperatures.

The use of granules of large sizes has been found in certain cases to greatly increase the life of recrystallized silicon carbide resistors. It has, however, been found that such resistors are frequently mechanically so weak as to require very careful handling to avoid breakage. The addition of a coating of fine material as described

below increases the strength of the resistor as indicated above and at the same time does not reduce the other desirable characteristics of the resistor.

5 As an illustration of the application of my invention, I take a slip made by mixing 80 per cent by weight of fine silicon carbide and 20 per cent of bentonite or a self-fluxing relatively insulating clay with sufficient water to keep the mixture 10 in suspension and apply this slip to the molded resistors by dipping the resistor in the slip or by spraying or brushing the slip onto the surface of the resistor. With resistors which are cured at a relatively low temperature, it is possible in some 15 instances to apply the glaze before the final curing of the resistor. Under ordinary circumstance, however, the coating should be applied after the resistor has been burned or cured, and it may then be baked onto the resistor in a furnace or 20 oven operated at a temperature sufficient to vitrify the binder used. With clay, this is from 2000 to 2500° F.

25 As another example of a suitable mixture, I may use a mixture of finely divided silicon carbide and bentonite together with finely ground sillimanite, clay or clay grog.

30 The silicon carbide used in the slip should be in a state of fine subdivision, preferably such as is obtained by mixing crushed silicon carbide with water and decanting the fine material after the mix has been allowed to settle a few seconds. Bentonite, as is well known, is a type of clay-like body which absorbs a large amount of water, 35 is somewhat fusible, and tends to produce a glazed surface when heated to 2500° F.

35 The glaze is particularly applicable to recrystallized silicon carbide resistors, and especially to resistors containing a substantial proportion of particles many times the size of the particles in the glaze itself. In the curing of a resistor by recrystallization, the strength of the article is believed to be due to the interlocking of the crystalline particles by a process of crystal growth. The silicon carbide is infusible, and with mixes 40 containing no appreciable proportion of fine material, it is difficult to secure a degree of self-bonding or crystal growth which will provide a high degree of strength. When my glazing material is applied, the strength of a coarse grit rod 45 can be increased to the point where it is com-

parable with a recrystallized resistor in which the original grit mix contained a substantial proportion of fine grit material. When my glaze is applied to a coarse grit resistor, the pores between the coarser particles in the original surface of the resistor are filled by the fine particles constituting the coating. The coating does not, however, penetrate to a material depth into the resistor.

5 While in the specific examples given, bentonite or fusible clay was used as a binder for the fine silicon carbide, other vitrifiable binders may be added or the impurities inherent in commercial fine silicon carbide such as silica, iron oxide, etc. may be utilized as a binder.

10 Although my glaze is very desirable for increasing the life and mechanical strength of silicon carbide resistors, it is also suitable for resistors composed of other carbides, and for the protection of resistors composed principally of carbon 15 or graphite.

15 I claim:

1. A silicon carbide heating element having a body portion composed mainly of coarse grains of silicon carbide and having a surface coating of 20 finely divided silicon carbide bonded with a heat hardened ceramic bond.

2. A silicon carbide heating element having a body portion substantially devoid of materials other than silicon carbide, the major portion of 25 said silicon carbide being relatively coarse, and having a surface coating of more finely divided silicon carbide which is bonded with a vitrifiable bonding agent.

3. A silicon carbide heating element having a 30 body portion composed mainly of coarse grains of silicon carbide and having a surface coating of finely divided silicon carbide bonded with a heat hardened ceramic bond, the silicon carbide particles in the body portion of the resistor being 35 many times the size of silicon carbide particles in the surface coating.

4. A recrystallized silicon carbide heating element, having a body portion composed substantially entirely of recrystallized silicon carbide, 40 and having a surface coating thereover, said surface coating being composed principally of finely divided silicon carbide and firmly attached to the resistor with a vitrifiable bonding agent.

ERNST HEDIGER. 50